

## UNITED STATES PATENT OFFICE

2,507,218

## MANUFACTURE OF HARD SINTERED ALLOYS

Marcel Oswald, Paris, France, assignor to Societe  
Le Carbone-Lorraine, Paris, France

No Drawing. Application July 30, 1947, Serial  
No. 764,899. In France July 4, 1941

Section 1. Public Law 690, August 8, 1946  
Patent expires July 4, 1961

6 Claims. (Cl. 75—137)

## 1

This invention relates to sintered hard alloys including zirconium carbide and other refractory carbides, such as the tungsten, titanium, vanadium, tantalum, etc., carbides. The agglomeration is in all cases obtained by means of a more fusible auxiliary metal or alloy. To all these alloys, zirconium carbide gives advantages due to its extreme hardness and to a greatly reduced coefficient of friction when cutting steels.

It has not been possible to introduce into industry the hard sintered alloys of zirconium carbide already known, because they have numerous blow-holes, especially when they are rich in zirconium carbide.

The process forming the subject matter of the invention does away with this disadvantage by making use of a new double zirconium and tungsten carbide represented by the formula  $Zr_3WC_4$  or of solid solutions of said carbide and the double titanium and tungsten carbide  $Ti_3WC_4$ .

The zirconium and tungsten double carbide is produced by mixing stoichiometrically calculated proportions of reducible compounds of zirconium and tungsten, as, for instance, the oxides  $ZrO_2$  and  $WO_3$  with the quantity of carbon necessary for reduction and carburisation. These substances in a fine powder are very carefully mixed and then heated in a vacuum furnace, so as to reach a temperature of at least  $2000^\circ C$ . The gases given off are pumped away as and when formed. A solid solution having the composition  $3ZrC.WC$  is thus produced, the atomic distribution of which is rearranged to convert the solid solution into the double carbide corresponding to the formula  $Zr_3WC_4$  by a suitable thermal treatment, namely slow cooling from  $1600^\circ C$ . to  $1000^\circ C$ . approximately. The double carbide has been prepared by reduction and carburisation at  $2200^\circ C$ .— $2300^\circ C$ . by maintaining the temperature above  $2100^\circ C$ . for about two hours, allowing to cool in an hour down to  $1600^\circ C$ . and then in eight to twenty-four hours from  $1600^\circ C$ . to  $1200^\circ C$ . and in two to four hours from  $1200^\circ C$ . to  $1000^\circ C$ . below  $1000^\circ C$ . the speed of cooling is no longer important. The double carbide forms a rather shiny metallic residue, of uniform coloration, loosely agglomerated and becoming well disaggregated by gentle crushing.

Incorporated in sintered alloys the double carbide described gives them the advantages of zirconium carbide, but with much greater facilities of application. The technical zirconium carbide always contains some protoxide. It is slightly wetted by metals of the iron family or their alloys, and the sintered alloys obtained are

## 2

always very fragile and porous. The double carbide on the contrary is well-wetted by metals and alloys of the iron group and gives satisfactory sintered alloys.

The results are still better if the double carbide  $Zr_3WC_4$  is replaced by a solid solution of this carbide with the double tungsten and titanium carbide. In these solutions, the atoms of titanium and zirconium take one another's places at random in the crystalline system in which they occupy the centres of the faces of the unit cells, the corners of said cells being left for the tungsten atoms. Solid solutions of simple carbides are already known, as, for instance, titanium carbide and molybdenum, or tungsten carbide, but not those between double carbides which are now.

In order to prepare solid solutions of the type  $(Ti, Zr)_3WC_4$ , reducible compounds of the three metals titanium, zirconium and tungsten are mixed in calculated proportions, so that for each atom of tungsten, this mixture contains three atoms of titanium and zirconium together. The required quantity of carbon is also incorporated to enable reduction and carburisation to be effected. These operations are carried out between about  $2000^\circ C$ . and  $2300^\circ C$ . according to the same process as for the double carbide  $Zr_3WC_4$ . In order to produce the required structure, cooling may take place at a suitable speed from about  $1600^\circ C$ . to  $1000^\circ C$ ., for instance, in from 10 to 30 hours and at any speed at other temperatures.

Solid solutions in particular have been prepared in which the atomic proportion of titanium and zirconium has one of the values 1:2, 1:1, 2:1. Increase in the proportion of titanium slightly reduces the hardness of the solid solution and increases the frictional coefficient of the sintered alloys, but to an admissible degree so long as the atomic ratio  $Ti:Zr$  does not exceed the value of 2.5 approximately.

By using a solid solution, briefly described as triple carbide containing two atoms of titanium per atom of zirconium according to the formula  $Ti_2ZrWC_4$ , the quality of the alloys with zirconium carbide is in the end improved, because the preparation is considerably facilitated, especially in the reduction and carburisation phase.

In order to prepare sintered alloys forming the subject matter of the invention, the zirconium carbide or the double carbide  $Zr_3WC_4$ , or a solid solution of the type  $(Zr, Ti)_3WC_4$ , is mixed with the other components: hard carbides, auxiliary metals or alloys, according to the known technical methods. Each of the constituents is in the form of a fine powder. After homogenisa-

tion, compression and sintering are carried out at a high temperature according to the usual methods. I shall now describe a few examples:

*Example 1.—Zirconium carbide, tungsten carbide and cobalt*

The compositions of this type are to be recommended, especially for proportions of carbide ZrC below about 20% by weight.

*Example*

|                                          |    |
|------------------------------------------|----|
| Double carbide of zirconium and tungsten | 13 |
| Tungsten carbide                         | 81 |
| Cobalt                                   | 6  |

It is preferable to prepare the mixture of tungsten carbide and cobalt by liberating the auxiliary metal and the refractory metal simultaneously in the nascent state by the action of a reducing and carburising gas such as coal gas so that there is simultaneously produced a condensation of pulverulent material which distributes itself in contact with the metallic grains and prevents them from growing; and then to incorporate the double carbide, make the mixture homogeneous, and press and sinter according to the known methods. Firing may take place in vacuo and at a temperature of 1600° C. to 1650° C. The alloys so obtained are slightly fragile but very hard.

*Example 2.—Zirconium carbide, titanium carbide, tungsten carbide, and a binding agent*

The mechanical resistance of alloys of zirconium carbide is greatly improved by incorporating with them titanium carbide in the proportion of at least one molecule of TiC per molecule of ZrC. The most convenient way is to employ a solid solution  $(\text{Zr}, \text{Ti})_3\text{WC}_4$  of the kind described. The following are two compositions:

|                                           | A  | B    |
|-------------------------------------------|----|------|
| Triple carbide $\text{Ti}_2\text{ZrWC}_4$ | 12 | 32   |
| Tungsten carbide                          | 82 | 61.5 |
| Cobalt                                    | 6  | 5.5  |
| Iron                                      |    | 1    |

The usual processes may be used, but there is advantage in preparing separately mixtures of tungsten carbide and binding metals in accordance with the process referred to in connection with Example 1 above: for (a) the whole of the tungsten carbide and cobalt; for (b) the tungsten carbide with 3.5 parts of cobalt and the whole quantity of iron. The compositions thus prepared are mixed with the triple carbide, and for (b) with the complement of cobalt, and then they are compressed and fired in an inert gas, in hydrogen or in vacuo between 1550° C. and 1600° C.

*Example 3.—Zirconium carbide—titanium carbide—tungsten carbide—tantalum carbide and binder*

The alloys prepared according to the preceding examples become more tenacious if they contain a percentage below about 8% of one or more carbides of metals belonging to the fifth periodic group; vanadium, columbium or tantalum. The three following compositions are respectively derived from those given in Examples 1 and 2, with additions of tantalum carbide and columbium carbide. The alloy (C) is preferably prepared

from the double carbide  $\text{Zr}_3\text{WC}_4$  and the alloys (D), (E) from the triple carbide  $\text{Ti}_2\text{ZrWC}_4$ .

|                   | C  | D     | E     |
|-------------------|----|-------|-------|
| Zirconium carbide | 6  | 2.5   | 7     |
| Titanium carbide  |    | 2.94  | 8.25  |
| Tantalum carbide  | 4  | 2     | 5     |
| Columbium carbide |    | 1     |       |
| Tungsten carbide  | 84 | 85.56 | 72.35 |
| Cobalt            | 6  | 6     | 5.5   |
| Iron              |    |       | 1     |

*Example 4.—Influence of vanadium and chromium*

The vanadium incorporated in the alloys of the foregoing types, diminishes or avoids blowholes and prevents enlargement of the grains. Harder and more tenacious alloys are then obtained, especially if a very small percentage of chromium is also added. The whole percentage of vanadium and chromium must be limited to less than 5% of the total weight and more often below 2%. The incorporation of vanadium and eventually of chromium, is carried out as described in the specification of my co-pending application Serial No. 764,901, filed July 30, 1947, now abandoned. It is possible to modify in this way the alloys above-mentioned, as examples, by the addition of vanadium and optionally of chromium, namely 1% of vanadium and 0.5% of chromium. Starting from the composition (B) of Example 2, the following alloy has been obtained and gives the best results:

|                                           |     |
|-------------------------------------------|-----|
| Triple carbide $\text{Ti}_2\text{ZrWC}_4$ | 32  |
| Tungsten carbide                          | 60  |
| Vanadium                                  | 1   |
| Chromium                                  | 0.5 |
| Cobalt                                    | 5.5 |
| Iron                                      | 1   |

The preparation of the powder to be sintered comprises, on the one hand, the manufacture of the triple carbide, and, on the other hand, the preparation of the mixture of the other constituents according to the aforementioned patent application, the mixture of the whole in the requisite proportions, pressing and firing. It is also possible to reduce the quantities of cobalt and/or iron introduced in the mixture of constituents other than the triple carbide, and to incorporate directly the remainder of the cobalt and/or of the iron in the final mixture as described in Example 2.

In cutting operations, especially at high speeds, the alloys of zirconium carbide reduce the frictional coefficient and render the operation almost noiseless, which is a new and unforeseen result. The noise in workshops is injurious to the auditory organs and to the nervous system; alloys with zirconium carbide, therefore, constitute desirable improvement.

In the above description it has been assumed that the zirconium carbide was prepared from an initial material free from hafnium. Now, most zirconium ores contain hafnium. Experience has shown that it is useless to separate these two elements; the small quantities of hafnium carbide eventually present exercise no harmful influence on the quality of the alloys. When there is hafnium present, the double carbide  $\text{Zr}_3\text{WC}_4$  is actually a solid solution  $(\text{Zr}, \text{Hf})_3\text{WC}_4$  in which the atoms of zirconium and hafnium are distributed in the same manner as Ti and Zr in the solid solution  $(\text{Zr}, \text{Ti})_3\text{WC}_4$ . If titanium carbide is incorporated with this solid solution, a solid

solution of the type  $(\text{Zr.Ti.Hf})_3\text{WC}_4$  is therefore obtained. In the whole description and in the claims the word zirconium designates either that metal or the natural and difficultly separable mixtures of zirconium and hafnium.

I claim:

1. Process of manufacturing sintered hard alloys, which comprises reducing and carburizing a finely powdered mixture of reducible compounds of zirconium and tungsten in the stoichiometric proportions of 3Zr to 1W, with carbon sufficient for reduction of said compounds to the metallic state and for carburization of the liberated metals, at a temperature between about 2000° C. and about 2300° C. while pumping off simultaneously liberated reaction gases, whereby to form a solid solution having the composition 3ZrC.WC, cooling the solid solution at a controlled slow rate through the temperature range from 1600° C. down to 1000° C. so as to rearrange the metallic atoms in the common crystalline lattice according to a superlattice, whereby to convert the solid solution into a cubic double carbide compound corresponding to the formula  $\text{Zr}_3\text{WC}_4$ , forming a homogeneous finely powdered mixture of an appreciable amount of said double carbide, at least one metal of the iron group, and at least one refractory metal carbide selected from the group consisting of tungsten carbide, titanium carbide, vanadium carbide, tantalum carbide, molybdenum carbide, chromium carbide and columbium carbide, compressing the mixture and sintering at a temperature between about 1200° C. and about 1600° C.

2. Process of manufacturing sintered hard alloys, which comprises reducing and carburizing a finely powdered mixture of reducible compounds of zirconium, titanium and tungsten in the proportions of 3 (Ti:Zr together) to 1W, with carbon sufficient for reduction of said compounds to the metallic state and for carburization of the liberated metals, at a temperature between about 2000° C. and about 2300° C., whereby to form a solid solution of zirconium, titanium and tungsten carbides, cooling the solid solution at a controlled slow rate through the temperature range from 1600° C. down to 1000° C. so as to rearrange the atoms of tungsten at the corners of the elementary cubes in the mixed lattice and form a solid solution of double carbides corresponding to the formulae  $\text{Zr}_3\text{WC}_4$  and  $\text{Ti}_3\text{WC}_4$  in which the atoms of tungsten occupy the corners and the atoms of zirconium and of titanium are distributed at random at the centres of the faces of the elementary cubes, forming a homogeneous finely powdered mixture of an appreciable amount of the cooled solid solution, at least one metal of the iron group, and at least one refractory metal carbide selected from the group consisting of tungsten carbide, vanadium carbide, tantalum carbide, molybdenum carbide, chromium carbide and columbium carbide, compressing the mixture and sintering at a temperature between about 1200° C. and about 1600° C.

3. Process as defined in claim 2, wherein the atomic ratio of titanium/zirconium is between 1:2 and about 2.5:1.

4. Process of manufacturing a sintered hard carbide composition of zirconium and tungsten, which comprises forming an intimate finely powdered mixture of oxides of zirconium and tungsten in the stoichiometric proportions of 3 $\text{ZrO}_2$  to 1 $\text{WO}_3$  with an amount of carbon sufficient for reduction of said oxides to the metallic state and for carburization of the liberated metals, heating

said mixture to a temperature of between about 2000° C. and about 2300° C. in vacuo while pumping off simultaneously liberated reaction gases, whereby to reduce said oxides and carburize the liberated metals, with the elimination of oxygen

5 from the reaction mass, to form a solid solution of tungsten carbide in zirconium carbide having the composition 3ZrC.WC, cooling said solid solution to 1600° C. in a period of one hour, then from 10 1600° C. to 1200° C. in a period of from eight to twenty-four hours, and then from 1200° C. to 1000° C. in from two to four hours so as to rearrange the metallic atoms in the common crystalline lattice to form a superlattice, whereby to convert said solid solution into a cubic double carbide compound corresponding to the formula  $\text{Zr}_3\text{WC}_4$ , forming a homogeneous finely powdered mixture of an appreciable amount of such double carbide, cobalt and tungsten carbide, compressing the last- 15 mentioned mixture and sintering at a temperature between about 1200° C. and about 1600° C.

5. Process as defined in claim 4, wherein the amount of said double carbide incorporated in said mixture last-mentioned is such as to provide 20 in the sintered composition a zirconium content calculated as  $\text{ZrC}$ , of less than about 10% by weight.

6. Process of manufacturing a sintered hard carbide composition of zirconium, titanium and tungsten, which comprises forming an intimate finely powdered mixture of reducible compounds of zirconium, titanium and tungsten in proportions such that said mixture contains two atoms of titanium and one atom of zirconium for each 30 atom of tungsten and with carbon sufficient for reduction of said compounds to the metallic state and for carburization of the liberated metals, heating said mixture to a temperature of between about 2000° C. and about 2300° C. in vacuo while pumping off simultaneously liberated reaction gases, whereby to reduce said compounds and carburize the liberated metals with the elimination of oxygen from the reaction mass, to form 35 a solid solution of zirconium, titanium and tungsten carbides, cooling said solid solution through the temperature range from 1600° C. down to 1000° C. in from ten to thirty hours so as to rearrange the atoms of tungsten at the corners of the elementary cubes in the mixed lattice and 40 form a solid solution of double carbides corresponding to the formulae  $\text{Zr}_3\text{WC}_4$  and  $\text{Ti}_3\text{WC}_4$  in which the atoms of tungsten occupy the corners and the atoms of zirconium and of titanium are distributed at random at the centres of the faces of the elementary cubes, forming a finely homogeneous mixture of cobalt, tungsten carbide and an amount of said solid solution of double carbides such as to provide in the final product a zirconium content, calculated as  $\text{ZrC}$ , of less than 45 50 about 10% by weight, compressing the last-mentioned mixture and sintering at a temperature between about 1200° C. and about 1600° C.

MARCEL OSWALD.

#### REFERENCES CITED

The following references are of record in the file of this patent:

#### UNITED STATES PATENTS

| 70 | Number    | Name          | Date          |
|----|-----------|---------------|---------------|
|    | 2,122,157 | Schwarzkopf   | June 28, 1938 |
|    | 2,137,144 | Sainderichin  | Nov. 15, 1938 |
|    | 2,170,432 | Schwarzkopf   | Aug. 22, 1939 |
|    | 2,188,983 | Padowicz      | Feb. 6, 1940  |
| 75 | 2,253,969 | Dawihl et al. | Aug. 26, 1941 |

**Certificate of Correction**

Patent No. 2,507,218

May 9, 1950

**MARCEL OSWALD**

It is hereby certified that error appears in the printed specification of the above numbered patent requiring correction as follows:

Column 3, line 9, for "20%" read 10%; column 4, line 8, in the table, fourth column thereof, for "72.35" read 73.25;  
and that the said Letters Patent should be read as corrected above, so that the same may conform to the record of the case in the Patent Office.

Signed and sealed this 14th day of November, A. D. 1950.

**[SEAL]**

**THOMAS F. MURPHY,**  
*Assistant Commissioner of Patents.*